

J. W. WEITZENKORN.

STEEL ALLOY.

APPLICATION FILED JAN. 25, 1918.

1,287,153.

Patented Dec. 10, 1918.



WITNESSES

J. Herbert Bradley.  
Francis D. Masson.

INVENTOR

Joseph W. Weitzenkorn  
by Christy and Christy  
his attorneys

# UNITED STATES PATENT OFFICE.

JOSEPH W. WEITZENKORN, OF WASHINGTON, PENNSYLVANIA, ASSIGNOR TO ELECTRIC REDUCTION COMPANY, OF WASHINGTON, PENNSYLVANIA, A CORPORATION OF DELAWARE.

## STEEL ALLOY.

1,287,153.

Specification of Letters Patent. Patented Dec. 10, 1918.

Application filed January 25, 1918. Serial No. 213,706.

To all whom it may concern:

Be it known that I, JOSEPH W. WEITZENKORN, residing at Washington, in the county of Washington and State of Pennsylvania, 5 a citizen of the United States, have invented or discovered certain new and useful Improvements in Steel Alloys, of which improvements the following is a specification.

My invention relates to alloys for structural articles made of steel. By such articles I mean to include structural steel elements entering into the manufacture of engines, machines, aeroplanes, marine torpedoes, etc., which elements, in proportion to 15 their weight, are required to possess great strength and toughness to resist repeated stresses of various characters.

The usual steel alloys from which such articles are manufactured, when heated to a high temperature and suddenly quenched or cooled, have high ultimate strengths and elastic limits, but they are exceedingly hard and brittle. To toughen such alloys the usual practice is to reheat them in order to draw or anneal them. While such prior alloys may be thus toughened, the toughness is attained at a very substantial sacrifice of strength.

The object of my invention is to provide 30 a steel alloy for such articles which will have both great strength and toughness, when quenched or cooled from a wide range of temperatures, or when drawn or annealed.

My invention proceeds upon my discovery 35 of a steel alloy which will not only have unusually great strength when cooled or quenched from a wide hardening range of temperatures, but will also possess great toughness, and which, when annealed or 40 drawn to further increase its toughness, will decrease but a relatively small amount in strength.

The alloy which I discovered, and which is characterized as just stated, contains not 45 more than about .60% of carbon, from about .50% to 1.50% of chromium, from about .10% to .50% of vanadium, and from about .50% to 1.25% of molybdenum. The alloy may contain additional substances either as alloying ingredients or as impurities.

While my invention is not limited to any specific mix, I have found that the best re-

sults may be obtained with a steel alloy containing about .35% carbon, 1.00% chromium, .15% vanadium, and from about .75% to 55 1.00% molybdenum.

Standard test specimens of an alloy of the composition just described were subjected to numerous tests to determine its physical properties. These specimens consisted 60 of 1½ inch round bars oil treated from 1600° F., machined to .505 inches in diameter, and subsequently drawn or annealed from various temperatures. The results of these tests have been carefully plotted on a curve sheet 65 which is reproduced on the accompanying drawing. The drawing shows the curves for the ultimate strength, elastic limit, percentage reduction of area and percentage of elongation in two inches of the specimens 70 when drawn or annealed from temperatures ranging from about 500° F. to 1400° F. There are also shown on the drawing the Shore and Brinell hardnesses of the alloy 75 when drawn from various temperatures.

It will be observed first that when the steel alloy is drawn from the relatively low temperature of 500° F., its ultimate strength is 250,000 pounds, its elastic limit 225,000 pounds and its reduction of area 35%. The 80 drawing of a steel from such relatively low temperature modifies but a slight amount the tensile strength and usual hardness of the steel when quenched from a relatively high temperature, say 1600° F. Hence it 85 will be seen that the steel alloy which I provide has an unusually high ultimate strength and elastic limit when quenched from a high temperature, and a very high percentage reduction of area when thus treated. 90

As the drawing temperatures are raised up to 1200° F. to further increase the toughness of the steel there is small loss of ultimate strength and elastic limit values as compared to prior dynamic steel alloys. 95 When drawn from 1200° F. the ultimate strength of the steel is about 187,000 pounds and the elastic limit about 173,000 pounds, while the unusual toughness of the steel when drawn from this temperature is indicated by the 60% reduction in area. 100

Dynamic articles made from the steel alloy which I have provided are exceedingly strong and tough in proportion to their

weight, and hence are particularly suitable for structures such as aeroplanes which are required to be light in weight.

I claim as my invention:

- 5 1. A steel alloy consisting of not more than .60% carbon, from about .50% to 1.50% chromium, .10% to .50% vanadium, and .50% to 1.25% molybdenum.
2. A steel alloy consisting of about .35%

carbon, 1.00% chromium, .15% vanadium, 10 and from about .75% to 1.00% molybdenum.

In testimony whereof I have hereunto set my hand.

JOSEPH W. WEITZENKORN.

Witnesses:

E. A. LUCAS,  
CLIFTON JAY.